

# UNITED STATES PATENT OFFICE.

HENRY L. COLES, OF HAMILTON, OHIO, ASSIGNOR TO NILES-BEMENT-POND COMPANY, OF NEW YORK, N. Y., A CORPORATION OF NEW JERSEY.

## COMPOSITION FOR THE TREATMENT OF CAST-IRON.

1,397,404.

Specification of Letters Patent.

Patented Nov. 15, 1921.

No Drawing.

Application filed July 10, 1920. Serial No. 395,187.

To all whom it may concern:

Be it known that I, HENRY L. COLES, a citizen of the United States, residing at Hamilton, in the county of Butler and State of Ohio, have invented certain new and useful 5 Improvements in Composition for the Treatment of Cast-Iron, of which the following is a specification.

This invention relates to the production of 10 cast iron and in particular to a composition to be added to the iron after it has been drawn from the cupola to avoid the effects drawn from the cupola to avoid the effects of sulfur and other ingredients which may cause red-shortness, blowholes and brittleness.

It is an object of the invention to provide a composition which may be added to cast iron in the form of a powder after or while the iron is being drawn from the cupola and 20 which will combine with the sulfur present in the iron and overcome its deleterious effects.

A further object of the invention is to provide a composition which may be used 25 conveniently and without complicating the process of smelting, molding or casting.

With the above and other objects in view my invention consists in the features of the 30 composition set forth in the following specification.

It is to be understood that the present showing discloses but one specific composition made in accordance with the present invention and that other compositions comprising substantially the same ingredients or the equivalents thereof are included within the spirit and scope of the invention as expressed in the appended claims.

The invention consists preferably in a 40 composition including an alloy of titanium, an alloy of manganese and a third compound or alloy which is included in the composition to aid in softening the iron. In the development of the invention I have used eight 45 parts of ferro-titanium, four parts of ferro-manganese and one part of ferro-silicon, but it is to be understood that the proportions of these compounds or alloys forming the composition may be considerably varied 50 without departing from the spirit of this invention. Furthermore, it is to be understood that other compositions of substances containing titanium, manganese and silicon may be used instead of the ferro alloys of

these elements and especially that the proportion of silicon, the function of which is to neutralize the hardening effect of the titanium present, may be varied or other elements substituted having a similar softening effect.

The alloys above mentioned or their equivalents are preferably mixed together in the proportions substantially as above indicated and the mixture then ground into powdered form. It may, however, in some instances, 65 be advisable to melt the mixture and, after allowing the mixture to cool, then crush it into a finely divided or powdered form.

In this powdered form the mixture is 70 added to the ladle and, as the iron is poured into the ladle the mixture becomes intimately mixed with the iron.

The sulfur present in the iron combines with the titanium forming titanium sulfid which forms throughout the molten mass, 75 the manganese also combines with the sulfur present forming manganese sulfid. As is well known the sulfur when combined with manganese is less detrimental to the quality of the iron than when it is combined directly with iron. There is a tendency, however, for the manganese sulfid to segregate from the iron in the form of large drops and, as these have little strength in themselves, they greatly weaken the iron.

The action of the elements titanium and manganese when combined in the proportions about as above specified has the effect of combining with all the sulfur present and causing the sulfur to permeate the entire 90 mass of iron in minute drops rather than to segregate in large drops of manganese sulfid which cause the iron to have an inferior quality.

The sulfur is not removed from the iron in 95 the form of slag, although, of course, some sulfur present may be removed in that manner. Practically the whole amount of sulfur is retained in the mass of iron and in so small particles and so intimately co-mingled 100 with the iron that the effects of the sulfur are not noticeable or detrimental.

One of the effects of the titanium present is to cause hardness of the iron and it is to overcome this hardening effect or tendency 105 of the titanium that a softening agent such as a compound of silicon, in the present instance ferro-silicon is added. Any other

softening agent acting in the same way may be substituted for the silicon.

The amounts of the composition to be used vary with variations in the amounts and proportions of sulfur and other impurities in the cast iron, and it is desirable that the relative quantities of these impurities be known before the composition is used, and the composition modified, if necessary, in accordance with the requirements of the particular iron being treated.

Furthermore, the proportions of the alloys forming my new composition may be varied for different characters of iron in which the impurities present are in different proportions. For instance, should the iron have manganese in its composition, the proportion of the manganese in the composition may be reduced accordingly. And in other characters of iron having a large amount of sulfur, an increased amount of both titanium and manganese may be required to neutralize its effects. An iron being treated which is soft may need but little silicon in the composition.

I have found in using a composition having the proportions above indicated that the amount of titanium in the final result should be about 0.2% and the manganese and titanium combined should, in the final result be at least 0.7%, and can be as high as 0.8%. With phosphorus in the iron between 0.7 and 0.8% the titanium should not be present in the final result above 0.2%, but with smaller amounts of phosphorus the percentage of titanium might be slightly increased.

What I claim is:

1. A composition for the treatment of iron, comprising a mixture of an alloy of titanium, an alloy of manganese and a softening agent.

2. A composition for the treatment of iron, comprising a mixture of ferro-titanium, ferro-manganese, and a softening agent.

3. A composition for the treatment of iron, comprising a mixture of ferro-titanium, ferro-manganese, and an alloy of silicon.

4. A composition for the treatment of iron, comprising a mixture of ferro-titanium, ferro-manganese, and ferro-silicon.

5. A composition for the treatment of iron, comprising a mixture of ferro-titanium,

ferro-manganese, and a relatively small quantity of a softening agent.

6. A composition for the treatment of iron, comprising a mixture of ferro-titanium, ferro-manganese, and a quantity of a softening agent sufficient to neutralize the hardening effect of the ferro-titanium.

7. A composition for the treatment of iron, comprising a mixture of a substance containing titanium, a substance containing manganese, and a quantity of a softening agent sufficient to neutralize the hardening effect of the titanium.

8. A composition for the treatment of iron, comprising a mixture of ferro-titanium, ferro-manganese, and a relatively small quantity of an alloy of silicon.

9. A composition for the treatment of iron, comprising a mixture of ferro-titanium, ferro-manganese, and a quantity of an alloy of silicon sufficient to neutralize the hardening effect of the ferro-titanium.

10. A composition for the treatment of iron, comprising a mixture of ferro-titanium, ferro-manganese, and a relatively small quantity of ferro-silicon.

11. A composition for the treatment of iron, comprising a mixture of ferro-titanium, ferro-manganese, and a quantity of ferro-silicon sufficient to neutralize the hardening effect of the ferro-titanium.

12. A composition for the treatment of iron, comprising a mixture of eight parts of an alloy of titanium, four parts of a compound of manganese, and one part of a softening agent.

13. A composition for the treatment of iron, comprising a mixture of eight parts of ferro-titanium, four parts of ferro-manganese, and one part of a softening agent.

14. A composition for the treatment of iron, comprising a mixture of eight parts of ferro-titanium, four parts of ferro-manganese, and one part of a compound of silicon.

15. A composition for the treatment of iron, comprising a mixture of eight parts of ferro-titanium, four parts of ferro-manganese, and one part of ferro-silicon.

In testimony whereof I hereto affix my signature.

HENRY L. COLES.